

## UNITED STATES PATENT OFFICE

2,191,652

## METHOD OF SEALING EARTH FORMATIONS

Andrew C. Hamilton, Jr., Dallas, Tex., assignor to  
 United States Gypsum Company, Chicago, Ill., a  
 corporation of Illinois

No Drawing. Application August 12, 1938,  
 Serial No. 224,637

6 Claims. (Cl. 61—36)

The present invention relates to improved methods for treating holes bored into the earth, as well as to the provision of footings and the like in earth-filled dams.

5 The present application is a continuation in part of my previously filed application Serial No. 203,815, filed April 23, 1938.

One of the principal objects of the present invention is a method for sealing off caves, holes, 10 water, and soft crumbly formations in the earth which may be encountered as a result of drilling holes into the earth, as for example when drilling a well. The method may also be applied to placing cementitious footings at the bottom of an 15 earth-filled dam, and the like, for the purpose of preventing seepage of water under the dam.

The invention may further be applied to the tamping of explosives in the bottom of a well or, for that matter, in any hole drilled into the earth.

20 In my aforementioned, previously filed, application Serial No. 203,815 I have described the invention particularly in connection with oil wells. When thus employed, the invention has particular applicability to the overcoming of the difficulty known in the industry as "loss of circulation" of the drilling mud used in the lubrication 25 of the drilling instruments, which mud also serves the function of bringing the drillings up out of the bore hole.

As is well known, when drilling a well it has 30 become customary to employ a special type of deflocculated mud which usually contains a weighting agent such as barium sulfate, this mud being pumped down into the well, particularly when using rotary drilling tools. The mud serves 35 three functions: first, to lubricate the drill; second, by reason of its weight, to keep back gas pressure and water pressure; and, third, to bring the cuttings and debris produced by the drilling to the surface. As the mud emerges to the top 40 of the hole being drilled it is usually sent to sumps or small lakes, where the drillings, etc. settle out, whereafter the remaining clarified mud is pumped back into the hole. When thus operating, everything will work satisfactorily provided there is a solid bottom to the hole so that 45 the mud can be pumped down into it, surrounding the drilling tool, the excess flowing back out of the hole at the top. However, if, when drilling, a cavity in the earth is encountered, difficulties may ensue. This is also true if a porous layer should be reached, through which the mud can escape. In any event, the mud fails to come back to the surface, preventing further operation 50 and causing financial loss. If, for example, a layer of gravel or similar porous material is encountered, the mud will seep out through it or even flow rapidly, depending upon the porosity of the structure. If there is ground water and 55 this is under pressure, this water may work up-

wardly through the bore hole and may even reach the surface, or may form a definite level therein, depending upon the pressure under which it is found. If there is much gas in the well, it may cause the water to be ejected with 5 considerable force. It has formerly been the practice, when encountering such difficulties, to sink a special casing in an attempt to get past or through the porous cavity, so that drilling can then be continued. This however requires the 10 use of a narrower casing, so that this can be lowered down inside the one already there. Obviously the further drilling of the hole would have to be with a smaller gauge. With the present invention, however, it is not necessary to employ a 15 smaller casing, because the cavity is sealed off by means of a cementitious material the setting time of which can accurately be controlled, but which is of such a nature that it is capable of forming 20 a readily pumpable slurry, readily introducible into the casing, so that it may flow out of the bottom of the casing and into the surrounding porous structure, setting at that point and plugging up the openings or pores in the structure.

It has been proposed in the past to lower bags 25 of a quick-setting cement into a bore hole and then to depend upon the water in the hole to unite with the cement and to form a plug. The bags of cement may either be left in place or may be ruptured and retrieved. In other words, in this prior process, solid pulverulent cementitious material was lowered into the hole and then allowed to set under the influence of the water present in the hole. This may be all right with water wells but would be very difficult if used in 30 very porous oil sand or something of that nature, because the oil would prevent the setting of the cement, which would simply pass out of the porous structure and be irretrievably lost. The same 35 thing is true if special types of cement are used in such a manner.

The specific embodiment of the present invention, so far as it relates to oil wells, therefore 40 differs from previous proposals in pumping into the well a sort of liquid slug or stopper consisting of a slurry of cementitious material which physically pushes water or other liquid ahead of it until it reaches the structure wherein it sets.

The basic principle of the invention is based 45 upon the fact that it is possible accurately to control the setting of a slurry of calcined gypsum or plaster of Paris, or similar calcium sulfate type of cement. It will readily be understood that if reliance were placed merely upon the slurry to obturate physically the openings in the structure, this alone would lead to no result, because unless the cement could be caused to set at the exact time when setting was desired, no plug would 50 form at all. This has been the great difficulty with the attempts to use Portland cement for 55 60

this purpose. It takes entirely too long for Portland cement to set, and furthermore the slurries made therewith are so heavy that they are not readily pumpable and certainly cannot be used in the manner in which the present invention is carried out.

Calcium sulfate,  $\text{CaSO}_4 \cdot 2\text{H}_2\text{O}$ , by itself is not a setting substance, but when it is heated to a suitable temperature it will lose some of its water, forming the hemihydrate,  $\text{CaSO}_4 \cdot \frac{1}{2}\text{H}_2\text{O}$ , which is a setting substance known in the industry under a number of names such as plaster of Paris, stucco, cement plaster, calcined plaster, gypsum plaster, etc. Ordinarily calcium sulfate hemihydrate when mixed with water will set very rapidly, say, on the order of from 4 to 5 minutes. It has therefore been customary to add to the calcined gypsum plasters various nitrogenous organic materials known as retarder, which retard the setting for a predetermined period. It is possible so to retard the setting of plaster of this kind that it will not set for many hours after being put in place, and the setting time can be controlled with great accuracy. Such retarders have been in use for many years and can be found described in textbooks on plasters, as, for example, Eckel's "Cements, Limes & Plasters", and in the patents to Melvin B. Church, No. 255,937, in which glue is described as a retarding material, and to George R. King, No. 368,594, in which glue is employed. Hydrolyzed keratinous materials such as hoofs and hair also have been widely used. Particularly applicable in the practice of the present invention is the set-stabilizing composition described by Alfred H. Gallagher in his Patent No. 1,683,539, in which waste animal hair is hydrolyzed with caustic soda under steam pressure, followed by the addition of lime. Gallagher also employing crystal-forming calcium sulfate accelerating material to balance the retarding effect of the hydrolyzed nitrogenous material so as to produce a plaster having a predetermined time of set. More recent patents along the same lines describing set-stabilized plasters having predetermined times of set are the patents to George D. King, Nos. 1,989,641; 2,078,198; 2,078,199 and 2,078,200.

In accordance with the present invention, a properly retarded calcium sulfate hemihydrate is employed. Let it be assumed that in the drilling of an oil well, for example let us say, for purposes of illustration, at a 1000-ft. level, difficulties are encountered by reaching a porous stratum or a cavity. Let it also be assumed that water tends to flow into the bottom of the well being drilled. When this condition is encountered, the present invention is brought into practice by an operation which is substantially as follows: The first thing that is done is to remove the drilling tools from the casing. Thereafter, by means of suitable pumps, water is rapidly pumped into the hole at such a rate that it will get into the hole faster than it will leave through the porous structure, so that the hole becomes filled up with water. In the meantime there has been prepared a slurry of calcium sulfate hemihydrate and water, say in the proportion of 100 parts by weight of the calcium sulfate hemihydrate and 30 to 80 parts by weight of water, which mixture forms a pumpable slurry. Knowing the length of time that it will take the slurry to get to the 1000-ft. level, sufficient retarder is mixed with the plaster before the water is added to retard it for about the time that it will take the prepared calcium sulfate slurry to reach the

porous stratum. Let it be assumed for purposes of illustration that it has been determined that it will take 45 minutes to do this. The plaster is therefore retarded so that it will begin to set about 45 minutes after it has first been mixed with water. The prepared calcium sulfate slurry having been made, the pumping of water is stopped, whereupon the water starts sinking into the bore hole. As this happens, the prepared slurry is introduced into the hole by pumps or other means, so that there will then be a column or slug of calcium sulfate hemihydrate slurry which follows the receding water down into the bore hole. Because this prepared slurry is properly retarded, it remains liquid; and when a sufficient amount of this slurry has been pumped in to form a plug of the predetermined size or the estimated size, water or mud is then pumped on top of the prepared slurry, forming another column on top of it. The force of this column continues to force down the slug or liquid plug of prepared slurry which then follows the water receding from the bottom of the bore hole until the prepared slurry arrives at the level of the porous stratum. Let it be assumed that 40 or 45 minutes have elapsed and that the prepared slurry is at the level of the porous stratum. Because of the retarder which has been calculated to cause setting at the end of 45 minutes, the previously liquid prepared slurry will now begin to set. At first it acts something like a starch gel and hence will not flow as freely as water, and as it gets into the small interstices of the porous stratum it will begin to obturate these porosities and within a few minutes will set to a solid. As soon as this takes place the pressure in the pipes through which the water or mud is pumped on top of the prepared slurry will greatly increase, which is an indication that the setting is taking place, whereafter the pumping can be stopped. Several hours are then allowed to elapse to insure the thorough setting and hardening of the plaster of the prepared slurry. Thereafter, the rotary drilling tools or other equipment are lowered into the well, and the drilling is resumed. As calcium sulfate when set is a soft and easily cut substance, it will take but a short time for the drills to find their way to the bottom of the hole; and as this is now surrounded by a set plug of gypsum or calcium sulfate plaster, there will be no loss of the mud, and the drilling can go on without further interruptions. If, later on, further porous strata should be encountered, the same procedure is repeated. In case merely an opening has been found, it may be necessary to estimate its approximate size. It may be only a small cavity, say a few hundred cubic feet, which causes the tool suddenly to drop and the mud to escape. If water is pumped into the hole until it overflows and this water has been measured or metered, some indication will be given of the size of the cavity. Therefore this water may be pumped out as much as possible and an amount of slurry corresponding in volume to the volume of the opening may be simply poured or pumped down into the hole until it extends to within a short distance from the bottom of the cavity and up into the casing. After enough time has elapsed for the setting of the material, which time can be calculated in advance, the drilling operation may be resumed, because then the cavity will have been filled up with the set calcium sulfate plaster.

The invention is of particular utility in connection with porous strata filled with gas, water, 75

or other liquids; and the method of application where a liquid slug of suitable substance is pumped down following a receding column of water and, if desired, followed by a succeeding column of mud or water, is the particular feature of the present invention and wherein it differs from the prior art, in which cementitious slurries such as Portland cement were merely pumped into the drilled hole in the hope that the cement would plug up the porosity. As already pointed out, such proposals usually failed because there was no way of controlling the set of the plaster at the exact time required, and therefore the cement slurry merely found its way out through the openings in the surrounding earth and was lost. This was sometimes overcome by pumping in enormous quantities of cement, which obviously is a very expensive expedient. However, with the present invention, by causing the setting of a slug of calcium sulfate hemihydrate slurry, only a small amount thereof is needed, and yet the hole is effectively shut off so that drilling may rapidly be recommenced.

In addition to being useful for the sealing off of oil wells, as just described, the invention is also applicable to the sealing of other holes which may have been drilled into the ground for other purposes. For example, recourse is often had to the drilling of holes into the earth for the purpose of reaching a stope in a mine for the purpose of ventilation. When drilling a hole for that purpose it often happens that ground water is encountered, which of course prevents further drilling of the hole or, if drilling were continued, would cause the water to be diverted into the mine. Obviously, therefore, it becomes necessary to shut off this ground water. This is accomplished in accordance with the teachings of the present invention in substantially the same way as described in connection with the sealing off of an oil well. In other words, advantage is taken of the fact that it has been found possible to produce a liquid pumpable slug of a potentially quickly setting substance such as calcium sulfate hemihydrate, which is pumped into the hole in the form of a slurry, the time of setting of the slurry being so controlled that the setting will take place about the time that the slug reaches the predetermined point in the hole.

In connection with oil-well sealing it is mentioned that calcium sulfate hemihydrate may be retarded to set in a predetermined time, but it should also be understood that in place of the retarders it may be advisable under some conditions to use set-accelerating salts or substances to speed the set of the gypsum. Such substances, well known in the art, are, for example, seed crystals of calcium sulfate dihydrate (either naturally or synthetically produced by metathesis from suitable salts), aluminum sulfate, sodium chloride, etc. Thus, for example, a plaster which has been retarded in manufacture may be found to be too slow setting, in which case accelerators may be added in suitable amounts; in fact, both accelerators and retarders may be used in order to produce predetermined setting time. Alternatively, it is possible to start with a set-stabilized plaster—which is well known in the art and can be purchased in the open market—having a setting time which has been predetermined by the manufacturer by the admixture with the plaster of both accelerating and retarding materials.

When the invention is used in connection with the drilling of ventilating openings or shafts into

mines, the operation of stopping off water and loose sand, gravel, etc., is commonly known as grouting. In the past, this has been attempted by the use of comparatively slow-setting hydraulic cements such as Portland cement; but as the setting time of these cements cannot be accurately controlled, they are often washed away by the water or escape through the loose formations without doing any good. By employing the present invention, however, a slug or liquid plug of calcium sulfate hemihydrate is forced into the hole under such conditions that, just about the time it reaches the point where it is desired to have it set, it will very rapidly set, thus sealing the hole at that point against water, loose sand, gravel, gas, etc. After the material has set, a hole may be drilled through it of the same size as the hole that is being drilled, whereafter the drilling may be resumed, continuing either until the desired stope has been reached or until further caves, water, gravel, etc., are encountered, when the invention can again be availed of.

A further utilization of the invention lies in the field of acidizing wells. As is well known, the acidizing of wells consists in pouring into the well, or forcing into it under pressure, a strong solution of an acid capable of dissolving the earthy formation at the bottom of the well, so as to open up the formation to permit oil from the surrounding earth formation to flow into the hole. An acid commonly used for that purpose is muriatic acid. However, if the bottom of the hole is very porous, such acid may work straight down without spreading out sufficiently to do any good in the area immediately surrounding the bottom of the hole. It has already been proposed to pour heavy liquids into the well for the purpose of producing a foot, which prevents the downward penetration of the acid, but such liquids are expensive and in many cases are quite inefficacious. However, a liquid slurry of calcined gypsum having a predetermined set can be forced into the well with the assurance that about the time it reaches the bottom of the well it will set and become hard. Some of it will also penetrate into the surrounding sand, particularly where there are crevices; and the operation can be so controlled that when acid is subsequently poured into the well it will tend to spread out laterally and act upon those earth formations which it is particularly intended to attack.

The present invention also has another very useful object, and that is its utilization in the sealing off of seepage flow under an earth-filled dam, levee, or dike. As is well known, dams are very often made merely by earth fill. Usually, such dams are based upon bedrock, upon which there is heaped a sufficiently high mass of earth, which is usually progressively narrowed toward the top. While this effectively stops water from flowing down a valley, it very often happens that water will, under the pressure of the water head accumulated behind the dam, force its way between the bedrock and the dam, despite the weight of the earthy matter lying on the bedrock. Such seepage can become quite serious and has been known to cause rupture of the dam. It has therefore been the practice in the past to attempt to place concrete or cement at the junction line between the earthy matter of the dam and the bedrock foundation thereof. If however water is already seeping, this procedure is ineffective, because the cement, which is applied in the form of a slurry, will be washed away by such water. The present invention however

solves this problem very effectively in the following manner:

Suitable holes are drilled vertically, or at an angle, through the dam until bedrock is reached. 5 There is then pumped into the holes—preferably under pressure, although if the holes are deep the pressure occasioned by the head of liquid may be sufficient—a thick slurry or slug of calcium sulfate hemihydrate, the setting time of which has 10 been so adjusted as to cause it to set substantially at the time when it penetrates from the bottom of the holes to some distance around the holes, at a point where the seepage is either taking place or is expected. This slurry upon setting will 15 therefore form a roughly circular mass at the surface of the rock foundation, whereafter it will be possible, if desired, to force ordinary cement in upon the wall of set gypsum, where it can then have ample time to harden without danger of being washed away by seepage water. This procedure 20 may be advisable, because calcium sulfate itself is not completely insoluble in water; and if it were used as the sole plugging means, it might be effective only for a number of years, because 25 the water might wash it away. However, the Portland cement behind it is not subject to being washed away by water, and by the time the set gypsum will have been washed away the concrete or cement will long since have reached its 30 maximum hardness and strength. In other words, the invention is used in such a manner that calcium sulfate hemihydrate of predetermined setting time is forced into the interface between the earth-filled dam or dike and the bedrock 35 between which it lies, to form a temporary bridge or dam at that point, serving as a retaining wall for subsequently applied ordinary Portland cement.

A still further embodiment of the invention 40 comprises its utilization for the tamping of explosives in the bottom of a well, as for example a water well or oil well. Thus, for example, a charge of nitroglycerin or similar explosive, together with a thereto attached primer and time 45 bomb, may be lowered into the bottom of a well; and thereafter a slug of calcium sulfate hemihydrate may be poured into the well, being so adjusted as to setting time that it will harden in the bore hole at the time it reaches the bottom of 50 the well or nearly the bottom of the well and will then set and thoroughly plug the hole. As calcium sulfate hemihydrate slightly expands on setting, it is particularly advantageous, because it insures a very tight tamping of the explosive. 55 There is thus little or no likelihood of the thus formed plug being blown or shot out of the hole. As the setting time can be controlled from thirty minutes to several hours, there will still be ample time to allow the calcium sulfate hemihydrate 60 to set before the time bomb goes off. Time bombs are usually adjusted to set off the charge of explosive at the end of eight to ten hours. When the explosive explodes, its force will be extended radially and downwardly around the hole, and 65 but little force will be exerted upwardly because of the resistance offered by the calcium sulfate dihydrate plug which resulted from the setting of the gypsum. After the charge has exploded, it is a simple matter to drill through the plug of 70 calcium sulfate dihydrate, because this is a soft substance which is very rapidly drilled through.

Other applications of the present invention will

readily be apparent to those skilled in the art of earth boring on the basis of the examples above given. While calcium sulfate has been described as the preferred setting material, the invention is not limited thereto, although it has been found that calcium sulfate hemihydrate is the most suitable, because it is easily controlled as to setting time, can be either accelerated or retarded, or both, and is also relatively inexpensive.

I claim:

1. The method of sealing an opening in the earth which comprises forcing into it a liquid slug or column of potentially hardenable calcined gypsum gauged with water and characterized by a definitely predetermined time of set until said 15 slug reaches the point in the opening where it is desired to seal the same and where the slug will then rapidly set to effect sealing of the opening.

2. The method of sealing off an opening in the 20 earth which comprises the steps of first filling it with water, then forcing into it a slug or column of potentially hardenable calcined gypsum gauged with water and characterized by a definitely pre- 25 determined time of set, permitting water to re- cede in the opening so as to cause the slug to travel downwardly in the opening until it reaches the point to be sealed, the time of setting of the calcined gypsum being so predetermined by admixture with sufficient set-controlling substances 30 as to cause it to set at about the time when the slug reaches the said point.

3. The method of preventing or minimizing seepage under an earth-filled dam, levee or dike which comprises drilling holes through the same 35 until bedrock is reached, then forcing into the holes and causing laterally to spread around the bottom of the holes a slurry of calcined gypsum having its setting time so controlled as to set in a roughly circular mass around the bottom of 40 the holes, and then forcing a slurry of Portland cement into the space between the mass of set gypsum and the bottom of the holes.

4. The process of sealing in or tamping an explosive in a hole in the earth which comprises 45 lowering a slug of calcined gypsum having a pre-determined time of set in admixture with water into the hole, whereupon the slug will set at a point between the explosive and the top or outlet of the hole.

5. The method of cementing off a well which comprises forcing into it a liquid slug or column of potentially hardenable calcined gypsum gauged with water and characterized by a definitely pre- 55 determined time of set until said slug reaches the point in the well where it is desired to seal the same and where the slug will then rapidly set to effect sealing of the well.

6. The method of sealing off a well which comprises the steps of first filling it with water, then 60 forcing into it a slug or column of potentially hardenable calcined gypsum gauged with water and characterized by a definitely predetermined time of set, permitting water to recede in the well so as to cause the slug to travel down the casing 65 of the well until it reaches the point to be sealed, the time of setting of the calcined gypsum being so predetermined by admixture with sufficient re- tarding as to cause it to set at about the time when the slug reaches the said point.

ANDREW C. HAMILTON, JR.